

## UNITED STATES PATENT OFFICE

GUSTAV REDDELIEN AND WERNER MÜLLER, OF LEIPZIG, GERMANY, ASSIGNORS TO AGFA ANSCO CORPORATION, OF BINGHAMTON, NEW YORK, A CORPORATION OF NEW YORK

## PHOTOGRAPHIC DEVELOPER AND PROCESS OF DEVELOPING PHOTOGRAPHIC MATERIALS

No Drawing. Application filed October 1, 1928, Serial No. 309,687, and in Germany November 21, 1927.

The present invention relates to new photographic developers, more particularly to developers comprising as a developing agent a compound of the general formula



wherein X represents a substituent other than a nitro-group and at least one X is a substituent other than hydrogen, and to the process of developing photographic materials 10 with these developers.

We found that photographic developers containing as a developing agent a N-mono-hydroxyethyl-derivative of nuclear substitution products of 4-amino-1-hydroxybenzene have remarkable advantageous properties. They are very stable in solid and in dissolved condition, are remarkably soluble and have the particular property of developing 15 the latent photographic image in a silver halide emulsion without formation of fog, even in solutions free from potassium bromide. N-mono-hydroxyethyl-derivatives of nuclear substitution products or homologues 20 of 4-amino-1-hydroxybenzene were hitherto unknown, the manufacture of them has been described in our co-pending application Serial No. 309,887, filed October 2nd, 1928, and consists in the condensation of nuclear substitution products of 4-amino-1-hydroxybenzene with a halogen-hydrin of glycol or with 25 ethyleneoxide. Suitable compositions for photographic developers in accordance with the present invention are obtained by mixing the developing agent with the ordinary developer ingredients.

Example 1.—1.17 gram of the sulfate of 4-hydroxyethyl - amino-2-chloro-1-hydroxybenzene,

40 9 grams of crystallized sodium sulfite and 5 grams of potassium carbonate are dissolved in 200 grams of water.

This developer has all the valuable properties referred to in the foregoing.

Example 2.—A developer of almost equal

activity to that of the developer described in Example 1 is made by dissolving in

200 grams of water  
1 gram of the oxalate of 4-hydroxyethylamino-3-methyl-1-hydroxybenzene  
3 grams of crystallized sodium sulfite and  
3 grams of potassium carbonate.

60

Example 3.—Another developer, which is very similar in action to the known 4-amino-1-hydroxybenzene-developer is made as follows:

Solution A: 3.65 grams of 4-hydroxyethylamino-1-hydroxybenzene - 2 - carboxylic acid and 5 grams of crystallized sodium sulfite are dissolved in 200 grams of water.

Solution B: 10 grams of potassium hydroxide are dissolved in 500 grams of water.

63

For use, 1 part of solution A, 1 part of solution B and 1 part of water are mixed together.

65

We claim:

1. A photographic developer containing together with other developer ingredients a compound of the general formula



wherein at least one X is a substituent taking the place of a hydrogen atom, which substituent, however, should not be a nitro group.

2. A photographic developer containing together with other developer ingredients a compound of the general formula



wherein 3 X's are hydrogen atoms and the 80 4th X is a substituent other than a nitro group.

3. A photographic developer containing together with other developer ingredients a compound of the general formula



wherein 3 X's are hydrogen atoms and the 88 4th X is an alkyl group.

4. A photographic developer containing

88

90

together with other developer ingredients a compound of the general formula



5 wherein 3 X's are hydrogen atoms and the 4th X is a methyl group.

5. A photographic developer containing together with other developer ingredients the oxalate of 4-hydroxyethylamino-3-methyl-1-hydroxybenzene.

10 6. A photographic developer containing together with sodium sulfite a compound of the general formula



15 wherein 3 X's are hydrogen atoms and the 4th X is a substituent other than a nitro group.

20 7. A photographic developer containing together with sodium sulfite a compound of the general formula



25 wherein 3 X's are hydrogen atoms and the 4th X is an alkyl group.

8. A photographic developer containing together with sodium sulfite the oxalate of 4-hydroxyethylamino-3-methyl-1-hydroxybenzene.

30 9. A photographic developer containing together with an alkaline solution of sodium sulfite and potassium bromide, a compound of the general formula



35 wherein 3 X's are hydrogen atoms and the 4th X is a substituent other than a nitro group.

10. A photographic developer containing 40 together with an alkaline solution of sodium sulfite and potassium bromide, the oxalate of 4-hydroxyethylamino-3-methyl-1-hydroxybenzene.

11. The process of developing photographic materials which comprises treating 45 the same with a solution containing a compound of the general formula



50 wherein at least one X is a substituent taking the place of a hydrogen atom, which substituent, however, should not be a nitro group.

55 12. The process of developing photographic materials which comprises treating the same with a solution containing a compound of the general formula



60 wherein 3 X's are hydrogen atoms and the 4th X is a substituent other than a nitro group.

13. The process of developing photographic materials which comprises treating

the same with a solution containing a compound of the general formula



wherein 3 X's are hydrogen atoms and the 4th X is an alkyl group.

14. The process of developing photographic materials which comprises treating the same with a solution containing a compound of the general formula



wherein 3 X's are hydrogen atoms and the 4th X is a methyl group.

15. The process of developing photographic materials which comprises treating the same with a solution containing the oxalate of 4-hydroxyethylamino-3-methyl-1-hydroxybenzene.

16. The process of developing photographic materials which comprises treating the same with a solution containing together with other developer ingredients a compound of the general formula



wherein 3 X's are hydrogen atoms and the 4th X is a substituent other than a nitro group.

17. The process of developing photographic materials which comprises treating the same with a solution containing together with other developer ingredients the oxalate of 4-hydroxyethylamino-3-methyl-1-hydroxybenzene.

18. The process of developing photographic materials which comprises treating the same with a solution containing sodium sulfite and a compound of the general formula  $\text{HO.C}_6\text{X}_4\text{.NH.CH}_2\text{.CH}_2\text{.OH}$ , wherein 3 X's are hydrogen atoms and the 4th X is a substituent other than a nitro group.

19. The process of developing photographic materials which comprises treating the same with an alkaline solution of sodium sulfite and a compound of the general formula  $\text{HO.C}_6\text{X}_4\text{.NH.CH}_2\text{.CH}_2\text{.OH}$ , wherein 3 X's are hydrogen atoms and the 4th X is a substituent other than a nitro group.

20. The process of developing photographic materials which comprises treating the same with a solution containing sodium sulfite, potassium carbonate, and the oxalate of 4-hydroxyethylamino-3-methyl-1-hydroxybenzene.

In testimony whereof, we affix our signatures.

GUSTAV REDDELIEN.  
WERNER MÜLLER.

125

130